

# UNITED STATES PATENT OFFICE.

CHARLES H. CURTIS, OF ARGOS, INDIANA.

## PROCESS OF PRESERVING WOOD.

1,022,064.

Specification of Letters Patent.

Patented Apr. 2, 1912.

No Drawing.

Application filed April 10, 1911. Serial No. 620,091

*To all whom it may concern:*

Be it known that I, CHARLES H. CURTIS, a citizen of the United States, residing at Argos, in the county of Marshall and State of Indiana, have invented certain new and useful Improvements in Processes for Preserving Wood; and I do hereby declare the following to be a full, clear, and exact description of the invention, such as will enable others skilled in the art to which it appertains to make and use the same.

This invention relates to a process for treating wood to preserve the latter by subjecting it to a solution composed of certain chemicals, and has for its object to render the wood stronger and more durable and to give it longer life.

In treating the wood by means of the solution employed, the wood is first sawed or carved into the desired shape or design. The sap and moisture is then driven out either by the heat of the sun or an ordinary dry kiln, or the ordinary vacuum pump apparatus may be employed. The wood is then ready for the second step of the process, which consists of a bath in a solution having the following ingredients and made in the following manner: Two parts of an alkali, preferably sodium carbonate (Na<sub>2</sub>CO<sub>3</sub>) are thoroughly mixed with one part of silica (SiO<sub>2</sub>), pure white sand, and ground dry by any ordinary mill which is capable of grinding finely. The mixture is then fused in an ordinary furnace forming a soluble alkali silicate



It is then allowed to cool and again ground to a fine powder. The mass is then dissolved in water (H<sub>2</sub>O) and chlorin (Cl) is then added. The solution is then ready to receive the wood to be treated, which should be immediately placed therein.

Chlorin (Cl) will unite with an equal volume of the hydrogen (H) of the water, forming hydrochloric acid (HCl); a sufficient quantity of chlorin (Cl) being added to form one pound of hydrochloric acid (HCl) for each pound of silica (SiO<sub>2</sub>) originally employed.

The solution may be injected into the wood by either the open tank or pressure methods now employed for such purposes.

When the cells and intercellular spaces of the wood are filled with the solution, the wood is placed in the hot sun or subjected

to a moderate heat in a dry kiln. The heat completes the union of the chlorin (Cl) and the hydrogen (H) in the cells and intercellular spaces of the wood, leaving silicon (Si) to unite with the two parts oxygen (O<sub>2</sub>), forming silica (SiO<sub>2</sub>), which remains in the wood, while hydrochloric acid (HCl) is, by means of heat, drawn from the wood, destroying at the same time a small portion of the wood fiber. The wood is again dried out, as described in the first step of the process, and then given a second bath in the solution, as described in the second step. The drying is again repeated and the wood subjected to a third bath. The steps of the process are repeated in regular order until the natural cells and intercellular spaces and the spaces made by the destruction of a portion of the wood fiber by the hydrochloric acid (HCl) are completely plugged or filled up with silica (SiO<sub>2</sub>). The wood at this stage of treatment is especially suitable for such uses as railroad ties, posts, telegraph and telephone poles, bridge timber, piling, etc., and for shingles and other building material.

Should a completely silicified wood be desired, the wood after being treated as above described, is subjected to a bath of sulfuric acid (H<sub>2</sub>SO<sub>4</sub>) under pressure, which more readily destroys the wood fiber than does the hydrochloric acid (HCl). It is removed from the solution when only a small portion of the wood fiber has been destroyed. It is then put through steps number one and two, thereby filling the spaces normally occupied by the destroyed fiber with the silica (SiO<sub>2</sub>), as the cells, intercellular and other spaces were filled in the first steps of the process. If desired, the treatment may be continued, using the sulfuric acid (H<sub>2</sub>SO<sub>4</sub>) bath until the wood is completely petrified.

During the above described preserving process all living organisms and fungi are killed and the finished product cannot be harmed by such wood destroyers.

The more porous and so called inferior woods after treatment by this process are rendered just as desirable as, if not more desirable than the high grade woods. Therefore, this process may be employed for preserving wood of all grades. And as mechanical abrasion is the chief destructive agent of a wood treated by this process, all wood so treated will be of great value for

all purposes for which wood is employed. Further, as the wood so preserved will have a practically endless life, the result will be an enormous annual saving of the rapidly diminishing timber reserves.

What I claim is:

1. The process of preserving wood, comprising preparing a solution by fusing together sodium carbonate and finely ground silica, cooling and pulverizing the frit, dissolving the same in water, treating said solution with chlorin gas; drying the wood by heat, immersing the dried wood in said solution, removing the wood from the bath and drying the same, and thereafter repeating the steps of immersing the wood in the solution and drying the same until the wood is impregnated to the desired degree.
2. The process of preserving wood, comprising preparing a solution by fusing together sodium carbonate and finely ground silica, cooling and pulverizing the frit, dissolving the same in water, treating said solution with chlorin gas; drying the wood by heat; immersing the dried wood in said solution, removing the wood from the bath and drying the same, and thereafter repeating

the steps of immersing the wood in the solution and drying the same until the wood is impregnated to the desired degree, thereafter immersing said wood in a bath of dilute sulfuric acid under pressure, to render the silica insoluble, and then again drying the wood by heating.

3. The process of preserving wood, comprising preparing a solution by fusing together sodium carbonate 2 parts, and finely ground silica 1 part, cooling and pulverizing the frit, dissolving the same in water, treating said solution with chlorin gas; drying the wood by heat, immersing the dried wood in said solution, removing the wood from the bath and drying the same, and thereafter repeating the steps of immersing the wood in the solution and drying the same until the wood is impregnated to the desired degree.

In testimony whereof I have signed my name to this specification in the presence of two subscribing witnesses.

CHARLES H. CURTIS.

Witnesses:

CHARLES W. WORTMAN,  
FRANK M. PICKERL.